

## UNITED STATES PATENT OFFICE

2,158,389

## LUBRICATING OIL

Charles Cole Towne, Beacon, N. Y., assignor to  
 The Texas Company, New York, N. Y., a corporation of Delaware

No Drawing. Application April 30, 1936  
 Serial No. 77,149

7 Claims. (Cl. 87—9)

This invention relates to the manufacture of an improved lubricating oil characterized by an increased viscosity index and other desirable properties.

5 The invention contemplates the preparation of mineral lubricating oil having an increased viscosity index by the addition to the oil of a minor proportion of the raffinate from an extraction with a wax anti-solvent of blown or polymerized fatty oils, such as blown rapeseed oil and polymerized fatty drying oils.

In the production of high grade lubricating oils, it is well known that a relatively small change in the viscosity of the oil between temperatures of say 100° F. and 210° F. is desirable. 15 In other words, it is advantageous for the oil to have a relatively flat viscosity temperature curve, which means that the oil has a high viscosity index as defined by Dean and Davis in their article 20 in Chemical and Metallurgical Engineering, vol. 36, page 618.

It has heretofore been proposed to add blown rapeseed oil or polymerized fatty oils to lubricating oil. However, the addition of substantial proportions of such oxidized or polymerized fatty oils is objectionable for high grade lubricants, such as motor oils, due to the increase in sludging characteristics, lack of oxidation stability and increased carbon residue. I have discovered that 25 this objection can be overcome and a superior product for this purpose obtained by extracting the oxidized or polymerized fatty oils with a solvent of the class of wax anti-solvents, and then employing the solvent insoluble portion or raffinate as the viscosity index improving material for 30 the lubricating oil. The materially increased effectiveness of the raffinate portion over the original oxidized or polymerized oil enables a much smaller proportion to be used to obtain the same effect, and the compounded oil possesses increased stability. Very satisfactory results have 35 been secured by extracting blown rapeseed oil or polymerized fatty drying oils, such as perilla, soy bean, and poppy seed, with a solvent such as acetone, or certain alcohols such as the propyl alcohols and the butyl alcohols. The extract or soluble portion contains material of comparatively small effectiveness in increasing the viscosity index of the lubricating oil, and in addition objectionable constituents which increase the sludging tendency or oxidation instability of the oil are 45 found in this extract. The insoluble portion or raffinate, on the other hand, constitutes the desirable material of high effectiveness for increasing viscosity index, and also imparts other desir-

able qualities such as increasing oiliness and film strength of the lubricant. The raffinate, after stripping of the retailed solvent, is added in a minor proportion to the mineral lubricating oil, generally in a proportion of about 1 to 10% on the weight of the oil. The raffinate may be added directly to the lubricating oil, or a solution of the raffinate in an aromatic solvent, such as benzol, may be prepared and added to the oil and the solvent removed by stripping.

By way of example, rapeseed oil was blown at elevated temperatures in the customary manner to a viscosity at 210° F. of 1785. 56 g. of this blown rapeseed oil were shaken vigorously with 800 cc. of acetone and allowed to settle. The lower insoluble layer was drawn off and heated to drive off the retained acetone. The upper layer was also heated to drive off the solvent thereby recovering the oil extracted by the acetone. 22 g. of oily material insoluble in acetone constituting 39% raffinate were obtained, a 61% extract.

The following results were obtained upon the addition of the indicated percentages of the acetone insoluble portion or raffinate and the acetone soluble portion or extract to a naphthene base oil:

|                                                  | Viscosity, °F. |      |                         | V. |
|--------------------------------------------------|----------------|------|-------------------------|----|
|                                                  | 100            | 210  | Zero, A. S. T. M. chart |    |
| 200 pale oil.....                                | 216            | 43   | 35000                   |    |
| Same+5% acetone extract of blown rapeseed.....   | 241            | 46   | 30000                   |    |
| Same+2% acetone raffinate of blown rapeseed..... | 257            | 47.5 | 27000                   |    |
| Same+5% acetone raffinate of blown rapeseed..... | 341            | 55.5 | 29000                   |    |

It is thus seen that 5% of the raffinate increases the viscosity index 100 points as against an increase of 51 points for the extract, while the stability of the oil blended with the raffinate is considerably improved over that blended with the extract. Moreover, 2% of the raffinate was found to give a greater increase in viscosity index than 5% of the extract.

Similar results are obtained by extracting polymerized fatty drying oils with acetone or alcohols mentioned, and employing the raffinate or insoluble portion as viscosity index improver for lubricating oils. The fatty drying oils polymerized or bodied in the customary manner by heating in an open kettle until they becom-

viscous as is well understood in the paint and varnish making art.

The following results show a comparison of the raffinate or insoluble portion of the oxidized or polymerized oils with the original polymerized or blown oils themselves, when added to various mineral lubricating oils:

|                                                                 | Viscosity, °F. |      |                               | V. I. |
|-----------------------------------------------------------------|----------------|------|-------------------------------|-------|
|                                                                 | 100            | 210  | Zero,<br>A. S. T. M.<br>chart |       |
| 100 pale oil                                                    | 530            | 52.5 | 350,000                       | 0     |
| Same+5% blown rapeseed                                          | 628            | 60   | 250,000                       | 46    |
| Same+2% acetone insoluble portion of blown rapeseed             | 638            | 60   | 275,000                       | 43    |
| Same+5% polymerized perilla oil                                 | 615            | 58.5 | 300,000                       | 36    |
| Same+5% acetone insoluble portion of polymerized perilla oil    | 704            | 63   | 225,000                       | 49    |
| Same+5% polymerized soy bean oil                                | 595            | 57   | 300,000                       | 28    |
| Same+5% acetone insoluble portion of polymerized soy bean oil   | 643            | 59.5 | 325,000                       | 38    |
| Same+5% polymerized poppy seed oil                              | 643            | 59   | 325,000                       | 33    |
| Same+5% acetone insoluble portion of polymerized poppy seed oil | 708            | 63   | 225,000                       | 48    |
| 100 pale oil                                                    | 310            | 46   | 120,000                       | -8.5  |
| Same+5% acetone insoluble portion of blown rapeseed oil         | 478            | 60   | 70,000                        | 85    |
| Same+2% acetone insoluble portion of blown rapeseed oil         | 373            | 51   | 90,000                        | 46    |
| 100 pale oil                                                    | 771            | 59.0 | 700,000                       | -2    |
| Same+5% acetone insoluble portion of blown rapeseed oil         | 1,110          | 79.5 | 525,000                       | 61    |
| Same+2% acetone insoluble portion of blown rapeseed oil         | 884            | 67   | 550,000                       | 38    |

Obviously many modifications and variations of the invention, as hereinbefore set forth, may be made without departing from the spirit and scope thereof, and therefore only such limitations should be imposed as are indicated in the appended claims.

I claim:

1. A lubricating oil of improved character comprising a mineral lubricating oil containing a minor proportion of the raffinate obtained from the extraction of a fatty oil selected from the group consisting of blown and polymerized fatty oils with a solvent selected from the group consisting of acetone, propyl alcohols and butyl alcohols.

2. A lubricating oil of improved character comprising a mineral lubricating oil containing, to the extent of around 1 to 10%, the constituents of an oil selected from the group consisting of blown and polymerized fatty oils and which are substantially insoluble in an extraction solvent selected from the group consisting of acetone, propyl alcohols and butyl alcohols and which are characterized by high viscosity index as well as resistance to oxidation and sludging. 10

3. A lubricating oil of improved character comprising a mineral lubricating oil containing a small quantity of the raffinate obtained from the extraction of a blown vegetable fatty oil with an extraction solvent selected from the group consisting of acetone, propyl alcohols and butyl alcohols. 15

4. The method of manufacturing an improved lubricating oil which comprises incorporating in mineral lubricating oil, to the extent of around 1 to 10%, the constituents of an oil selected from the group consisting of blown and polymerized fatty oils and which are substantially insoluble in an extraction solvent selected from the group consisting of acetone, propyl alcohols, and butyl alcohols and which are characterized by high viscosity index as well as resistance to oxidation and sludging. 25

5. A lubricating oil of improved character comprising a mineral lubricating oil containing 1 to 10% of the raffinate from an extraction of blown rapeseed oil with a solvent selected from the group consisting of acetone, propyl alcohols and butyl alcohols. 30

6. A lubricating oil of improved character comprising a mineral lubricating oil containing 1 to 10% of the raffinate from an extraction of polymerized perilla oil with a solvent selected from the group consisting of acetone, propyl alcohols and butyl alcohols. 35

7. A lubricating oil of improved character comprising a mineral lubricating oil containing 1 to 10% of the raffinate from an extraction of polymerized poppy seed oil with a solvent selected from the group consisting of acetone, propyl alcohols and butyl alcohols. 40

CHARLES COLE TOWNE.